

July 3, 1928.

1,675,666

W. M. SHOEMAKER, JR.

METHOD OF MAKING FIBER BOARD

Filed Dec. 27, 1926

3 Sheets-Sheet 1



INVENTOR

William M. Shoemaker Jr.

By Cyrus V. Anderson  
ATTORNEY

July 3, 1928.

1,675,666

W. M. SHOEMAKER, JR

METHOD OF MAKING FIBER BOARD

Filed Dec. 27, 1926

3 Sheets-Sheet 2



INVENTOR  
BY William M. Shoemaker Jr.,  
Cyrus N. Anderson  
ATTORNEY

July 3, 1928.

1,675,666

W. M. SHOEMAKER, JR

METHOD OF MAKING FIBER BOARD

Filed Dec. 27, 1926.

3 Sheets-Sheet 3



INVENTOR

William M. Shoemaker Jr.  
Cyrus N. Anderson  
ATTORNEY

## UNITED STATES PATENT OFFICE.

WILLIAM M. SHOEMAKER, JR., OF KENNETT SQUARE, PENNSYLVANIA, ASSIGNOR TO NATIONAL VULCANIZED FIBRE COMPANY, OF WILMINGTON, DELAWARE, A CORPORATION OF DELAWARE.

## METHOD OF MAKING FIBER BOARD.

Application filed December 27, 1926. Serial No. 157,219.

- The present invention relates to the manufacture of fiber sheets or fiber board quite generally known in the trade as "vulcanized fiber", in which a plurality of thin sheets of cellulosic material may be united to form a single sheet; or a single sheet may be employed which may be rolled up over a heated drum or cylinder to produce a sheet of the thickness required.
- 10 Heretofore in the manufacture of fiber board the practice has been, as far as I am aware, to subject thin sheets preferably of unsized cotton cellulose paper, to the action of a suitable metallic salt such as zinc chloride in solution in water by passing the said sheets through such a solution having a strength of about 70° Baumé and at a temperature ranging from ordinary room temperature to about 35° C., and conducting the sheets from the said solution directly to and between heated drums or cylinders by means of which the said sheets are subjected to pressure and heat and union thereof effected to form a single sheet.
- 15 In the manufacture of fiber board it is necessary, after the impregnation of the sheets with a suitable solution, usually consisting of a suitable chemical in water, that heat be applied thereto. Heretofore the
- 20 heated pressure drums or cylinders or other pressure means, between which the sheets have been compressed to effect union thereof, have been relied upon for supplying the heat necessary to be applied to the said sheets. By this method the heat is applied directly only to the outer surfaces or sides of the top and bottom plies or sheets of the plurality of sheets being united. In order that there may be no question but that
- 25 the sheet or sheets which enter into the final product shall have been subjected to the same treatment it is desirable that heat be applied to each sheet separately preferably, though not necessarily, to both sides thereof
- 30 simultaneously. As a result of so applying the heat and thereby effecting uniformity of application of heat to each sheet a product having uniform texture throughout is assured.
- 35 The general object, therefore, of the present invention is to provide a novel method by the employment of which a plurality of sheets of cellulosic material may be united to form a fiber board or fiber sheet having improved structural characteristics and qualities.
- 40 Other and further objects of the invention are to provide a novel method by the employment of which both sides of each of a plurality of sheets of cellulosic material which may be united to form a single sheet may be subjected to the action of heat at a temperature requisite to and for the manufacture of fiber board, or "vulcanized fiber" as it is generally called in the trade; 45 to provide a novel method wherein and whereby the respective plies or sheets of cellulosic material are each subjected to the same degree of temperature; to provide a novel method wherein and whereby the 50 plies or sheets which form the interior of the final product shall have been subjected to the same degree of temperature as the sheets forming the outer sides or surfaces thereof; and to provide other improvements 55 as will be set forth hereinafter.
- 55 As a result of the application of heat at the temperature required to the separate sheets which are to be united I have discovered that a more satisfactory product 60 may be obtained than has been obtainable by the employment of the methods heretofore known and employed in the manufacture of fiber board.
- 65 In describing the method embodying my invention it is preferable that reference be made to an apparatus which may be employed for handling the sheets of cellulosic material and effecting the necessary treatment thereof and the uniting of the same 70 to form relatively thick sheets of fiber board. Accordingly, therefore, I have invented and designed an apparatus of novel construction which may be employed in the carrying out of the method invented by me 75 and to which reference will be made in connection with the description of the said method.
- 80 In the accompanying drawings I have illustrated one form of apparatus embodying the novel means invented by me for forming one or a plurality of sheets into fiber board or "vulcanized fiber" and to which I shall refer in detail in the following description.
- 85 In the drawings.
- 90 Fig. 1 is a view in side elevation of a portion of a machine or apparatus by the

employment of which the improved method invented by me may be practised;

Fig. 2 is a view partly in side elevation and partly in longitudinal section of the remaining portion of the said machine or apparatus;

Fig. 3 is a view taken in a plane parallel with the opposing sides of a heat unit constituting a part of the means for heating separately and individually the sheets of cellulosic material, the union of which is to be effected, the said view showing a portion of the heating means in plan; and

Fig. 4 is a transverse sectional view taken on the line 4—4 of Fig 3.

In the drawings I have shown a magazine 10 or supply of plies or sheets of cellulosic material, a tank 11 containing a suitable chemical such as zinc chloride or other suitable metallic salt or other chemical in solution in a suitable solvent, such as water, for impregnating the said sheets, a heating means 12 for the application of heat at the requisite temperature simultaneously to both sides of each of the chemically treated plies or sheets, and a compressing means 13 wherein the plies or sheets are superposed and merged by pressure into a single sheet. This sheet, after the usual treatment to effect removal of the chemical with which the respective sheets were impregnated or saturated and after having been dried, becomes what is known as fiber board or "vulcanized fiber." The plies or sheets usually consist of cotton cellulose but may consist of cellulose obtained from other sources and may also consist of a mixture of cellulose obtained from different vegetable sources.

The magazine 10 preferably is of open frame construction having journals 14 suitably mounted on side bars 14<sup>a</sup> to rotatably support the rolls 15 of paper (cellulose sheets) which depend in number upon the number of sheets or plies to be used to form the finished product; that is, the fiber board sheet. Thus, if a five-ply material is to be made only five rolls 15 will be used; while if a fifteen-ply material is to be made there will be fifteen rolls 15 in operation.

50. The solution 16 (preferably of zinc chloride or other suitable metal salt) of suitable strength, say around 70° Baumé, in the tank 11 is provided in sufficient quantity to insure the complete immersion of the maximum number of plies or sheets which may be employed. The temperature of the solution as employed may range from ordinary room temperature to a temperature of about 35° C. One end of the tank 11 is of arc shape as shown in order to provide clearance to permit lateral movement of the pivoted spacing guide cage 17 toward the left in Fig. 2 of the drawings, and upwardly to a position above the tank 11 to facilitate the insertion 60 or threading of the plies or sheets 21 between

the spaced guides 18 and 20 provided in two series located in two spaced upwardly converging planes, as shown in Fig. 2. Each guide of one series is located in a position horizontally opposite that of the corresponding guide in the other series. After the sheets 21 have been threaded through the cage 17 underneath opposing guides 18 and 20 and said cage is lowered into the tank 11 as shown in Fig. 2 the said sheets, as they 70 travel forward, are held in spaced substantially parallel relation to each other while in and as they pass through the bath or solution 16. The parallel relationship is unimportant but it is important that they be held spaced from each other. It will be noted that the upper plies or sheets 21 remain in the said bath or solution for a shorter period than do the successive lower plies or sheets. It follows, therefore, that the speed of travel 80 or movement of the sheets through the bath or solution must be such as to allow sufficient time for the necessary impregnation of the uppermost sheets. This is a practical matter 85 and may be readily controlled or provided 90 for.

To provide for the operation of the cage 17 it is mounted upon a swinging frame 22 which includes lifting arms 23 and a chain hoist 24 whereby it can be swung out of and 95 above the bath 16 for the purpose previously stated.

In order to effect uniform heating of each plies or sheet 21, after its passage through the bath 16 and prior to the union of the sheets, 100 the heating means 12 is provided. In its preferred form the said means consists of a plurality of heating units each of which comprises plates 25 and 27 spaced from and in parallel relation to each other to form a wide thin chamber as indicated in Figs. 2, 3 and 4 of the drawings. For supplying a heating medium to the respective chambers formed by the spaced plates 25 and 27 I have provided in each chamber a tubular 105 structure comprising side members 30 and 31 which are connected by cross-wise extending tubes 32 having openings 32<sup>a</sup> in the opposite sides thereof. For heating the respective units steam is supplied to the pipes of the tubular frame structure of each unit and escapes through the openings in the cross tubes 32 and through openings 33 in the inner sides of the side tubes 30 and 31 into the chamber between the plates 25 and 27 and is condensed so that the said chamber becomes filled with water at a temperature sufficient to supply the heat to be applied to the respective sheets 21 as they travel 115 through the passageways 26 between the adjoining units. The temperature to which the said sheets may be subjected may range from about 38° C to about 93° C. The upper surface of the plate 25 of each unit 120 preferably is slightly convex as shown. As 130

the respective sheets 21 are conducted through the passageways 26 they contact with the convex surfaces of the plates 25 of the respective units. The adjoining units 5 are located close together so that the spaces 26 through which the sheets travel are quite narrow. The heat, in the construction shown, is applied to the lower sides of the respective sheets as they pass through the pass- 10 sageways 26 by conduction from the plates 25 with which they are in contact, while to the opposite sides thereof heat is applied by radiation from the plates 27 of adjoining units. The plates 27 of adjoining units are 15 so close to the upper sides of the sheets as they travel through the spaces 26 that each side of each sheet is subjected simultaneously to heat at substantially the same temperature. The sheets being quite thin it fol- 20 lows that the particles thereof are affected in substantially equal degree. The result of this is that the characteristics of the respective sheets are the same or substantially the same so that when they are combined into a 25 single sheet a product having uniform and improved characteristics and qualities as compared with products as heretofore manufactured is the result.

Although it is preferred to apply heat to 30 both sides of each sheet as above described, it is to be understood that my invention comprehends the application of heat to one side only of each sheet. When the said sheets are thin it is apparent that such application usually would accomplish the re- 35 sult desired.

In the case of sheets of cellulosic material 40 of relatively low absorbtivity usually characterized as "hard", it will be found that upon the passage of the same through the solution the outer portions of the opposite sides thereof will be sufficiently impregnated to cause efficient union thereof upon their 45 passage between the compression cylinders or drums 35 and 36. It may be that the portions of such sheets between the said outer portions upon the opposite sides thereof will not be impregnated, or only partially im- 50 pregnated, but such a condition will not interfere with the efficient union of adjoining sheets. All of the sheets which may be 55 passed through the solution and thereafter united will have been subjected to identical treatment and will have substantially the same characteristics.

The respective heating units are supported in spaced relation to each other to provide the passageways 26, to which reference has been made, by the interconnection of the tubes (through which the heating medium is supplied to the respective units) between the said units, and the heating means 12 as a whole is supported by the common supporting frame 34.

65 In undergoing the treatment as thus far

described impregnation of the sheets with the salt solution or other chemical solution in the tank 11 and gelatinization thereof have been effected. They are now in condition and ready to be superposed and subjected 70 to pressure to effect union thereof to form the product desired, namely, fiber board or "vulcanized fiber" as it is generally called.

For effecting union of the sheets which have been treated as hereinbefore described, 75 they are conducted from the heating means to the pressure means 13 comprising the heated cooperating pressure drums or cylinders 35 and 36. By reason of the fact that the individual plies or sheets have been 80 subjected already to the action of heat by the heating means 12 it is not necessary that these drums or cylinders 35 and 36 be maintained at as high a temperature as heretofore has been the practice. The sheets to be 85 united are conducted over the drum or cylinder 35, around a portion thereof, and between the said drums or cylinders 35 and 36 and thereby subjected to heavy pressure in known manner whereby union thereof is 90 effected to form a sheet having a combined thickness of the united plies or sheets. The sheet or board formed by the uniting of the said plies or sheets is led away from the 95 pressure drums as indicated at 37 and may be cut into sections of such length as may be desired. These sections then are subjected to the usual treatment to effect removal of the chemical with which the respective sheets 100 were impregnated as they moved or passed through the solution 16 in the tank 11. After the removal of such chemical, usually zinc chloride, the sheets are dried. However, the present invention is not concerned 105 with the treatment of the sheets after they leave the pressure means 13.

In the methods and apparatus heretofore employed in the manufacture of fiber board or "vulcanized fiber" the thickness of the sheets constituting the final product which might be manufactured has been restricted or limited. Such restriction and limitation have been due to the fact that the heated pressure drums or cylinders corresponding 110 to those designated 35 and 36 in the drawings have been relied upon to furnish the heat necessary to be applied to the respective sheets in order that satisfactory union thereof might be effected. As already indicated, 115 when the pressure drums or cylinders were relied upon to supply the required heat the application thereof has been made only to the outer sides of the outer plies. It is apparent, therefore, that such a method and such an apparatus would be restricted and limited as to the thickness of the fiber board sheet of uniform quality which might be produced thereby.

120 The method and apparatus of the present invention are not circumscribed by such re- 125

strictions and limitations because of the application of heat at the required temperature to each sheet of a plurality of sheets which are to be united prior to the bringing of the 5 same together between the pressure cylinders or drums of the compression means by which union thereof is effected.

An important and essential feature of my invention consists in the application of heat 10 to the respective sheets which are to be united, preferably simultaneously to both sides of each sheet, after the same has been impregnated with the solution of salt or other chemical 16 and prior to the bringing 15 of the said sheets together and the subjection of the same to pressure within the compression means 13 to effect union thereof.

While I have illustrated a plurality of plies or sheets treated and united to form a 20 single sheet of fiber board it will be understood that my invention may be employed in the formation of a fiber board sheet from a single thin sheet of cellulosic material of proper character by winding the same up on 25 the drum or cylinder 36 to obtain the required thickness. The removal of such sheet from the drum or cylinder may be effected in known manner by slitting the same.

It is to be understood that the invention is 30 not limited to apparatus of the specific construction illustrated herein and that the said invention is susceptible of embodiment in apparatus of other forms of construction than that shown, and also that the method 35 invented by me may be practised and carried out by means other than that shown in the present apparatus.

Having thus described my invention, what I claim and desire to secure by Letters Patent is:

1. The method of forming a fiber sheet from a plurality of sheets of cellulosic material, which consists in impregnating a plurality of said sheets of cellulosic material 45 with a suitable chemical, thereafter subjecting each sheet of cellulosic material to the action of heat at the requisite temperature, and thereafter superposing said sheets of cellulosic material and effecting union thereof.

2. The method of forming fiber board from a plurality of sheets of cellulosic material, which consists in subjecting the respective sheets to the action of a suitable

metallic salt in solution to effect impregnation thereof, thereafter subjecting the respective sheets to heat at the requisite temperature while holding the said sheets in spaced relation to each other, and thereafter superposing the said sheets and applying pressure thereto to effect union thereof.

3. The method of forming fiber board from a plurality of sheets of cellulosic material, which comprises the subjection of the said sheets to the action of a suitable chemical solution in water to effect impregnation thereof, causing the said sheets to move through a zone of heat at requisite temperature, holding the said sheets while moving through said zone in spaced relation with respect to each other, thereafter bringing the said sheets together, and subjecting the same to pressure to effect union thereof.

4. The method of forming fiber board, which consists in passing a plurality of sheets of cellulosic material through a water solution of a suitable metallic salt, conducting the said sheets in spaced relation to each other away from the said solution and while so spaced applying heat at requisite temperature simultaneously to both sides of each sheet, and thereafter bringing the said sheets together and effecting union thereof.

5. The method of forming fiber board, 85 which consists in conducting a plurality of cellulosic sheets in spaced relation to each other through a solution of zinc chloride, thereafter supporting said sheets in spaced relation to each other and applying heat at 90 requisite temperature to each individual sheet to effect the necessary gelatinization, and thereafter bringing the said sheets together and effecting union thereof to form a single sheet.

6. The method which comprises the steps of impregnating a web of cellulosic material with a suitable gelatinizing agent, moving said web through a heat zone wherein heat at substantially the same temperature is 100 applied simultaneously to both sides thereof, and laminating said web, the steps being performed successively and continuously.

Signed at Wilmington, county of New Castle, State of Delaware, this 23rd day of December, 1926.

WILLIAM M. SHOEMAKER, JR.